

[54] **METHOD OF FABRICATING COMPOSITE  
MULTI-METALLIC BILLETS USEFUL FOR  
METAL WORKING OPERATIONS**

[75] Inventor: Alvin L. Hurst, Lower Burrell, Pa.

[73] Assignee: Aluminum Company of America,  
Pittsburgh, Pa.

[22] Filed: Oct. 10, 1972

[21] Appl. No.: 296,006

[52] U.S. Cl. 29/420, 29/191.2, 29/DIG. 31

[51] Int. Cl. B22f 3/04

[58] Field of Search. 29/420, 420.5, DIG. 31,  
29/DIG. 47, 191.2, 182.1, 182.2; 75/208 R, 226[56] **References Cited**

## UNITED STATES PATENTS

|           |         |                |            |
|-----------|---------|----------------|------------|
| 3,010,196 | 11/1961 | Smith et al.   | 29/420.5   |
| 3,066,403 | 12/1962 | Brauchler      | 29/191.2 X |
| 3,279,917 | 10/1966 | Ballard et al. | 29/DIG. 31 |
| 3,285,714 | 11/1966 | Davies et al.  | 29/182.1   |
| 3,373,003 | 3/1968  | Schreiner      | 29/182.2   |
| 3,678,567 | 7/1972  | Manilla et al. | 29/420.5   |
| R20,460   | 8/1937  | Jeffrey        | 425/112 X  |

|           |         |                    |          |
|-----------|---------|--------------------|----------|
| 2,517,902 | 8/1950  | Luebkeman          | 264/91   |
| 2,695,231 | 11/1954 | Causley            | 75/208 R |
| 3,146,099 | 8/1964  | Teja               | 75/208 R |
| 3,335,001 | 8/1967  | Drew et al.        | 75/208 R |
| 3,391,444 | 7/1968  | Haller             | 29/420.5 |
| 3,447,230 | 6/1969  | Bargainnier et al. | 29/420.5 |

Primary Examiner—Richard J. Herbst

Assistant Examiner—D. C. Reiley, III

Attorney—Robert E. Isner et al.

[57]

## ABSTRACT

Method of fabricating compacted composite multi-metallic billets for metal working operations having at least two discrete metal constituents disposed in predetermined desired positional disposition therein. Included therein is the formation of at least a pair of discrete powdered metal receiving cavities of predetermined configuration within a deformable shell, introduction of powdered metal therein and isostatic compaction to predetermined desired density without appreciable change in the relative physical disposition of the metals, one to the other.

6 Claims, 12 Drawing Figures





**METHOD OF FABRICATING COMPOSITE  
MULTI-METALLIC BILLETS USEFUL FOR  
METAL WORKING OPERATIONS**

This invention relates to the fabrication of compacted powdered metal billets for metal working operations and particularly to the fabrication of composite billets formed of at least two discrete metal constituents of differing metallurgical characteristics selectively disposed in predetermined desired positional disposition both internally and externally thereof.

The fabrication of certain types of non-planar composite multi-metallic products, such as rods, bars, tubes or shapes, from two or more discrete metals or metal alloys of differing metallurgical characteristics by conventional practices is both relatively expensive and of limited utility because of the difficulties attendant formation of properly contoured and constituted starting billets that permit direct production of the desired composite multi-metallic product of predetermined configuration and character by extrusion or other conventional fabrication operation.

The invention may be briefly described as an improved method of fabricating compacted composite multimetallic billets for metal working operations formed of at least two discrete metal constituents of differing metallurgical characteristics selectively disposed in predetermined desired positional disposition both internally and externally thereof. In its broader aspects, the subject invention includes the positioning of an elongate hollow partition member of a first predetermined cross-sectional configuration within a closed end deformable shell of a second predetermined cross-sectional configuration and of at least substantially commensurate length therewith, with the dependent end of such partition member disposed in abutting relation with the closed end defining wall portion of the deformable shell member to cooperatively define at least a pair of discrete powdered metal receiving cavities of predetermined cross-sectional and longitudinal configuration therein. Finely divided particles of metal of differing metallurgical character are then selectively introduced into said receptacles to substantially fill the same. After removal of such partition member, which serves to introduce the partition engaging surfaces of said metal particles into intimate interfacially engaged relation at a defined interface therebetween, the deformable shell and its contents are subjected to isostatic compaction, as by application of hydrostatic pressure, to compact said finely divided metals to a predetermined desired density without any appreciable change in the relative physical positional disposition of such metals, one to the other. In its narrower aspects, the subject invention is particularly directed to the fabrication of composite multi-alloy billets for the extrusion of selectively clad aluminum base alloy products and includes the positioning of an elongate thin walled hollow core member of a first predetermined cross-sectional configuration within a closed end deformable shell of predetermined cross-sectional configuration and of at least substantially commensurate length therewith, with the open end of the core member disposed in abutting relation with the closed end defining wall portion of the shell member to form a pair of discrete aluminum base alloy powder receiving cavities therein. Subsequent to the selective introduction of discrete finely divided aluminum base alloy powders of differing met-

allurgical character into such cavities, the core member is axially removed and the deformable shell member and its contents is hydrostatically subjected to cold isostatic compaction to produce a self-supported compact 5 or billet having said discrete aluminum base alloy powders compacted to predetermined density without appreciable change in the relative physical positional disposition thereof permitting, without further treatment such as sintering or the like, extrusion thereof to form 10 a composite or clad product of predetermined internal and external character.

Among the advantages of the subject invention is the permitted simple and inexpensive formation of composite multi-metallic billets of predetermined discrete 15 internal and external configuration to permit the direct production of composite multi-metallic products of predetermined character in a subsequent metal working operation. Another advantage of the subject invention is the permitted fabrication, at markedly reduced 20 cost and expense, of compacted composite billets of aluminum base alloy powders of predetermined desired configuration suitable for direct utilization in subsequent metal working operations. A further advantage of the subject invention is the permitted fabrication of cold compacted composite multi-alloy billets for the extrusion of selectively clad aluminum base alloy products from at least two discrete aluminum base alloy 25 powders of differing metallurgical character that dispenses with the need for sintering and which permits production of an acceptably bonded clad product of desired internal and external configuration upon subsequent extrusion thereof.

The primary object of this invention is the provision 30 of an improved method for fabricating composite multi-metallic billets of predetermined desired internal and external configuration for metal working operations.

Another object of this invention is the provision of an improved method for fabricating composite multi-metallic billets from at least two discrete powdered 35 metal constituents of differing metallurgical character and having such differing metal constituents disposed in predetermined desired configuration both internally and externally thereof.

A further object of the invention is the provision of an improved method for forming composite multi-alloy billets from discrete aluminum base alloy powders for fabrication of selectively clad aluminum base alloy products that dispenses with the need for sintering 40 thereof.

Still another object of the invention is the provision of an improved method of fabrication of selectively clad extruded aluminum base alloy products from discrete aluminum base alloy powders having predetermined desired external and internal configuration at 45 the bonded interface thereof.

Other objects and advantages of this invention will be apparent from the following portions of the specification and from the appended drawings which schematically illustrate, in accordance with the mandate of the 50 patent statutes, certain presently preferred operations deemed by the inventor to incorporate the principles of this invention.

Referring to the drawings

FIGS. 1(a) through 1(e) schematically illustrate, in vertical section, features of a preferred sequence of 55 steps employable in the fabrication of multi-metallic billets in accord with the principles of this invention.

FIGS. 2(a) through 2(e) are horizontal sections as taken on the line 2-2 through FIGS. 1(a) through 1(e), respectively.

FIG. 3 is a horizontal section, similar to FIG. 2(c), schematically illustrative of fabrication of an extrusion billet having a core portion of a cross sectional configuration different from that of the outer or cladding portions.

FIG. 4 is a horizontal section, similar to FIG. 2(c), schematically illustrative of a rectangularly shaped multi-metallic billet for sheet fabrication.

Referring to the drawing, and particularly to FIGS. 1 and 2, there is schematically and exemplarily illustrated features of certain of the sequenced steps employable, in accord with the principles of this invention, in the fabrication of composite multi-alloy billets for the extrusion of selectively clad aluminum base alloy products. To the above ends, and as shown in FIG. 1(a), an open ended, elongate and thin walled partition member conveniently in the form of a cylindrical tube 10 of circular cross-section is co-axially disposed within a closed end deformable shell 12 of a second predetermined cross-sectional configuration. In the illustrated structure, the shell 12 is also of circular cross-section to ultimately form a cylindrical billet and is of a length generally commensurate with that of the partition tube 10. Such co-axial disposition of the open ended tube 10 within the closed end shell 12 with the dependent open end 14 thereof disposed in abutting relation with the closed end defining wall portion 16 of the deformable shell 12 results in the formation of a pair of discrete powder receiving cavities or receptacles 18 and 20 therewithin. The core or interior cavity 18 is entirely defined by the tube 10 and the wall 16 and is definitive of a cylinder of circular cross-section. The second cavity 20 is conjointly defined by the positional disposition of the outer wall surface of tube 10 relative to the inner wall surface of shell 12 and in the illustrated embodiment comprises an annulus of uniform thickness.

The outer deformable shell 12 is suitably of the type conventionally employed in hydrostatic compaction apparatus and may be formed of rubber or deformable resinous material, such as polypropylene, polyvinyl chloride and the like. The removable thin walled partition member 10 may be constituted by any suitable material of sufficient strength and rigidity as to resist deformation and displacement during the powdered metal filling operations as hereinafter will be described, and may be conveniently formed of aluminum or steel sheet or of relatively rigid resinous material.

After selective positioning of the partition member 10 within the deformable shell 12 as described above to define metal receiving cavities of predetermined desired configuration, and as shown in FIG. 2(b), a first discrete metallic constituent in the form of finely divided aluminum base alloy powder 22 of a first predetermined metallurgical character is selectively introduced into the cavity 18 to substantially fill the same. Either simultaneously or sequentially with respect thereto, a second discrete metallic constituent in the form of finely divided aluminum base alloy powder metal 24 of a second and different metallurgical character from that of the first metallic constituent is selectively introduced into the second cavity 20 to substantially fill the same. When so filled, the outer shell 12 and its contents may be subjected to light jarring or tamping so as to effect a preliminary gravity induced

compaction of the introduced metal particles within the cavities 18 and 20.

For the purposes of this application the terminology "discrete metals" and "different metallurgical character" and the like is intended to broadly encompass metal containing constituent materials having any ascertainable metallurgical difference therebetween and which are capable of ultimately providing an acceptably bonded interface therebetween and thus to include utilization of dissimilar metals, such as copper, steel or aluminum as well as alloys, such as utilization of two or more recognized alloys of aluminum. Also, as used herein, the term "aluminum base alloy" is intended to encompass all such alloys in which the major proportion, i.e., 50 percent or greater, is aluminum.

Following the above, and as shown in FIG. 1(c), the partition member 10 is then removed from the shell 12 by lineal displacement along its longitudinal axis, as indicated by the arrow 26, in such a manner as to effect a minimal disturbance of the metal particles disposed in proximity to the inner and outer surface thereof. Such displacement of the partition tube 10 serves to introduce the particles of the discrete metal powders therefore disposed in abutting facing relation with the inner and outer surfaces of such partition tube 10 into intimate interfacially engaged relation, as illustrated by the dotted lines 28. Complete removal of the partition tube 10 results in the formation of a composite and uncompacted multi-metal powder preform as illustrated in FIG. 2(d) consisting of a cylindrical core of a first aluminum base alloy 22 disposed within a surrounding annulus of a second aluminum base alloy 24. The deformable shell 12 is then conventionally sealed, as by the cap 30, and, after evacuation, subjected to hydrostatic pressure in a suitable press to effect isostatic compaction of the shell 12 and its composite multi-metal powdered fill by conventional techniques as for example generally disclosed in U.S. Pat. Nos. 3,313,871 and 3,608,026. Such isostatic compaction operates to effect a marked increase in the density of the compact and in a uniform reduction of its size, as generally illustrated in FIG. 1(e), without appreciable change in the relative physical positional disposition, both internally and externally, of the now compacted aluminum base alloys 22a and 24a, one to the other.

In the preferred practice of the subject invention, as indicated above, compacted composite multi-alloy billets are formed of aluminum base alloys for the extrusion of selectively clad aluminum base alloy products.

By way of illustrative example, and for the fabrication of cylindrically shaped billets of about 7 1/2 inch outside diameter and about 12 inches long, the core defining elongate partition tube 10 may be filled with 5056 alloy powder and the cladding defining annular cavity 20 filled with 6253 cladding powder. After removal of the core tube 10, sealing of the shell 12 and evacuation thereof, the shell 12 and its contents were subjected to unit hydrostatic pressures in the order of 32 ksi. The resulting cylindrically shaped compacts were of the character described above and were sufficiently self-supporting to permit machining and normal handling thereof preparatory to extrusion. These composite compacts were subsequently heated to extrusion temperature which is not only well below any sintering temperature therefore, but also concomitantly provided a degree of degassing thereof. While at extrusion temperature, the compacted billets were convention-

ally extruded into satisfactory 2 7/8 inch round corner, square alclad bars. The resulting product appeared to have interparticle bonds of nominally the same strength as those present in extrusions from composite billets fabricated in accord with conventional practice. Subsequent examination of such extruded product showed the maintained presence of a distinct line of demarcation between the two aluminum base alloy constituents thereof and without any ascertainable intermixing or infiltration of one alloy into the other. The particles of the two alloys at the interface appear to be joined to each other in the same manner as would be effected by particles of the same alloy.

FIG. 3 illustrates the permitted utilization of an elongate, thin walled partition member 40 of rectangular cross-section within a deformable shell 42 of circular cross-sectional configuration. Operations as described above will result in the provision of a composite billet having a rectangular core portion 44 of a first metal constituent and a discrete outer or cladding portion 46 of a second metal constituent of a generally annular configuration but with dissimilarly shaped inner and outer surfaces thereof.

FIG. 4 schematically illustrates the application of the principles of this invention to the fabrication of a composite rectangularly shaped billet. In this embodiment, an elongate thin walled planar partition member of rectangular cross-section 50 is coaxially disposed in uniform spaced relation within a larger and rectangularly shaped deformable shell 52 and serves to cooperatively define a rectangular central or core cavity 54 and a surrounding peripheral cladding cavity 56 of generally uniform thickness. Introduction of discrete aluminum base alloy powders of differing metallurgical character into the core cavity 54 and into the cladding cavity 56, followed by removal of the partition 50 and isostatic compaction, as described above, results in the formation of a compacted fillet of rectangular configuration particularly adapted for rolling operations in the fabrication of clad sheet product.

Billets of the above character and of about 6 inches square by about 19-19 1/2 inch long have been readily fabricated by the described technique from 5056 and 6253 aluminum base alloy powders and employing unit hydrostatic pressures of about 21-23 ksi.

Having thus described my invention, I claim:

1. In the formation of composite multi-metallic billets for the fabrication of selectively clad metal products, the steps of

positioning an elongate, hollow open-ended and relatively thin-walled core member of a first predetermined configuration within a closed-end deformable outer shell member of larger transverse di-

mension and of substantially commensurate length therewith with one open end of said core member disposed in abutting relation with the closed-end defining wall portion of said shell member to define a plurality of powdered metal receiving cavities therein,

introducing a first finely divided metal powder material into a cavity defined by and disposed intermediate said core member and said shell member in sufficient quantity to substantially fill the same, introducing a second finely divided metal powder material of metallurgical characteristics different from those of said first powder material into a second cavity disposed within and defined by said hollow core member in sufficient quantity to substantially fill the same,

axially removing said core member from said shell member to introduce the particles of said first and second discrete metal powders disposed in abutting relation with the inner and outer surfaces of said core member into intimate interfacially engaged relation without substantial disturbance in the physical positional disposition thereof relative to each other,

sealing said deformable shell member.

and isostatically said sealed deformable shell member and its contents to hydrostatic pressure to compact said powder metal contents thereof to a predetermined desired density without appreciable change in the relative physical positional disposition of said first metal material to said second metal material.

2. The method as set forth in claim 1 wherein said first and second finely divided metal powder materials are aluminum base alloys.

3. The method as set forth in claim 2 including the step of heating said compacted multi-alloy billet to extrusion temperature and extruding the same to form a selectively clad aluminum base alloy product of predetermined configuration.

4. The method as set forth in claim 1 wherein said core member and said shell member are of similar cross-sectional configuration.

5. The method as set forth in claim 1 wherein said core member and said shell member are of different cross-sectional configuration.

6. The method as set forth in claim 2 wherein said thin walled core member and said deformable shell member are of circular cross-sectional configuration, to provide a compacted billet having a cylindrical core and an annular layer of cladding metal enclosing the same.

\* \* \* \* \*

UNITED STATES PATENT OFFICE  
CERTIFICATE OF CORRECTION

Patent No. 3,780,418 Dated December 25, 1973

Inventor(s) Alvin L. Hurst

It is certified that error appears in the above-identified patent and that said Letters Patent are hereby corrected as shown below:

Column 1, line 23, "The" should read -- This --. Column 2, line 66, "empolyable" should read -- employable --. Column 3, line 12, "drawing" should read -- drawings --. Column 4, line 65, "therefore" should read -- therefor --. Column 5, line 38, "fillet" should read -- billet --; line 42, "inch" should read -- inches --. Column 6, line 26, after "isostatically" insert -- subjecting --.

Signed and sealed this 12th day of November 1974.

(SEAL)

Attest:

MC COY M. GIBSON JR.  
Attesting Officer

C. MARSHALL DANN  
Commissioner of Patents